

Feb. 17, 1931.

L. G. FIRTH

1,792,581

METHOD OF MAKING NONPOROUS ARTICLES

Filed Aug. 12, 1929

Fig. 1.



Fig. 2.



Fig. 3.



Fig. 4.



Fig. 7.



Fig. 6.



Fig. 5.



INVENTOR

L. Gerald Firth  
Byers, Stebbins, Parmenter &  
Blanka  
1,792,581

## UNITED STATES PATENT OFFICE

LOUIS GERALD FIRTH, OF PITTSBURGH, PENNSYLVANIA, ASSIGNOR TO FIRTH-STERLING STEEL COMPANY, OF MCKEESPORT, PENNSYLVANIA, A CORPORATION OF PENNSYLVANIA

## METHOD OF MAKING NONPOROUS ARTICLES

Application filed August 12, 1929. Serial No. 385,255.

This invention relates to a method of making nonporous articles.

Ingots of steel or other metals or alloys are now usually cast in molds having a substantially square cross-section. The ingot molds are sometimes provided with hot-tops through which the metal is poured into the mold, the hot-tops being used to keep the metal in liquid condition, thereby tending to decrease the amount of shrinks, pipes, and porosity of the cast ingot. Even with the use of hot-tops, however, the ingots are somewhat porous and for certain purposes it is necessary to scrap a large proportion of the ingot and use only that portion of the ingot which is substantially entirely free from porosity, segregation and shrinks. In making pistons for pneumatic rock-drills, valve seats and valves which are to be subjected to great pressures, or for airplane work, or other similar usages, it is necessary that the metal be substantially free from defects such as segregation, shrinks, or porous structure.

My invention is particularly adapted where it is necessary that the ingot be substantially free from the defects above mentioned. The usual process of casting ingots as practiced at the present time is to pour in such a way that the last portion to cool is at the top of the ingot and may be discarded. However, in any given cross section of an ingot at right angles to its longitudinal axis, the last portion to cool is the extreme center. It is probable that the central 5% to 15% of this cross section cools almost simultaneously, i. e., the solidification is progressive from the sides of the mold up to a certain point, at which point more or less simultaneous freezing takes place. It is this central 5% to 15% which contains the greater part of the segregated impurities and gases. This central portion also usually cools progressively from the bottom of the ingot to the top and it is customary to discard the upper portion or pipe end which, generally speaking, is the last portion to cool. It is impracticable, however, under present practice to discard the whole of that central axis or core which extends from the bottom to the top of the ingot and

which contains the steel last to cool in each horizontal plane.

In my invention, I not only discard the top portion of the ingot, according to common practice, but I also sever the ingot longitudinally and discard that portion in each horizontal plane which was the last to cool. It is in this respect that my invention differs radically from present day practice. The approximate amount of this last cooled portion to be removed according to my process is from 10% to 30% of the original weight of the ingot, this being taken mainly from the central portion of the casting. When a very high degree of perfection is required, as much as 50% of the original weight may be removed from the central portion. This can be regulated by cutting the ingot nearer or further from its central axis.

In my reference to "horizontal planes" and "longitudinal axis" I refer to ingots cast upright according to the usual practice, but my invention can also be applied when the ingot is cast with the longitudinal axis sloping or horizontal. In accordance with my invention, the ingot is cast in a mold having recesses formed therein which form flanges on the ingot extending outwardly from the body portion of the ingot. Any shrinks, pipes, or porous structure which may be present in the ingot are in the central portion thereof, and the flanges are free from such defects. The flanges are then separated from the relatively porous body portion and are worked by rolling or other shaping methods to form the desired articles.

In the accompanying drawings, which illustrate several present preferred embodiments of my invention;

Figure 1 is an elevation of an ingot mold;

Figure 2 is a section on the line II-II of Figure 1, showing the ingot in the mold;

Figures 3 and 4 are sections similar to Figure 2, but showing ingots having four and five flanges, respectively;

Figure 5 is a section similar to Figures 2, 3, and 4, but showing another modification;

Figure 6 is a horizontal section of one of the flanges formed on the ingot, after the

55

60

65

70

75

80

85

90

95

100

flange has been separated from the body portion of the ingot; and

Figure 7 is a perspective view of a rock-drill piston.

Referring more particularly to Figs. 1 and 2 of the drawings, there is shown an ingot mold 2 which is generally triangular in shape. The mold is formed of sections 3, 4, and 5, which are bolted together by bolts 6 and nuts 7. The mold is provided with recesses 8 extending radially from a central recess 9. The recesses 8 taper outwardly from the central portion of the mold, for a purpose hereinafter described.

In casting an ingot in the illustrated mold, the metal is poured in the usual manner, preferably through a hot-top. The metal flows into the recesses 8 to form an ingot having a central body portion 10 and flanges 11 extending therefrom. Each of the flanges 11 has its three outer sides cooled by the mold. The side of the flange 11, which is connected to the central portion 10 of the ingot, remains hot for a longer time than the other sides of the flanges which contact with the mold sections. The cooling action of the ingot takes place first on the sides exposed to the mold sections so that the flanges 11 are formed without shrinks, porous spots, or segregation. The only porous portion of the ingot is the central portion 10.

The flanges 11 are then separated along the lines 15 from the central portion of the ingot which was the last portion to cool. After separation the flanges, which are entirely solid, are rolled, forged, or otherwise shaped into the desired articles.

The ingot shown in Figure 3 is similar to the ingot of Fig. 2, except that in Fig. 3 the ingot has four flanges 11a instead of three. An ordinary mold 20 of substantially square cross-section can be converted into a mold embodying my invention by inserting filler blocks 21 in the corners of the mold in order to form a mold having recesses 8a which form flanges 11a on the ingot. When the mold shown in Fig. 3 is used for casting the ingot, the flanges 11a are separated along the lines 15a from the central portion of the ingot.

In Fig. 4 there is shown a mold having five recesses 8b, which form an ingot having five flanges 11b extending radially therefrom. My invention contemplates the formation of an ingot having any number of flanges formed thereon.

In Fig. 5 another form of ingot mold is shown. This mold has recesses 8c formed therein, which form the flanges 11c on the ingot. It also has recesses 25 provided in the mold which form flanges 26 on the ingot. When a mold of this shape is employed, the flanges 8c are separated from the remainder of the ingot along the lines 15c and only the two flanges 11c are worked to form the desired articles. The recesses 25 in the mold

and the corresponding flanges 26 formed on the ingot are provided in order to cause the shrinks and segregations to take place as indicated at 27, and in order that the flanges 11c will be free from such defects.

The illustrated molds are made in sections which are bolted together in order to free the molds. If desired, solid molds may be employed instead of split molds, and any number of recesses may be provided in the molds to form a corresponding number of flanges on the ingots.

The recesses 8, 8a, 8b, and 8c, preferably slope outwardly from the central portion of the mold. In Fig. 6 there is illustrated a flange 11 formed in the mold illustrated in Fig. 2. As above stated, the flanges 11 are substantially free from porosity and segregation. However, there is a small portion 12 of the flange which is not quite as dense as the remaining portion of the flange. This is due to the fact that the portion 12 is the last to cool. In order to make the density of the billet rolled from the flange 11 absolutely uniform, the flanges are cast having a slight taper outwardly from the central portion of the ingot. The inner portion 30 of the flange accordingly is subjected to greater work than the outer portion 31 when the flange is rolled. The greater amount of work to which the portion 30 is subjected gives the rolled billet substantially uniform density throughout.

After rolling, forging, or otherwise shaping the flange 11, it is formed into the desired article.

A piston 35 for a rock-drill is illustrated in Fig. 7. Pistons made according to my invention are free from porosity, shrinks, and other defects and are particularly adapted for the work which they have to perform. If a piston for a rock-drill is slightly porous, it is likely to crack under the strain imposed by the terrific impact of the piston against the other parts of the rock-drill.

My invention is especially useful in the production of alloy steel articles which are expensive and in which it is desired to reduce to a minimum the portion of the ingot which it is necessary to discard because of its porous character.

If desired, the ingot may be cast into molds which are rotated in order to force the metal from the central portion of the mold into the recesses which form the flanges on the ingot.

I have illustrated and described several preferred forms of the invention. It is to be understood, however, that the invention may be otherwise embodied within the scope of the following claims.

I claim:

1. The method of making non-porous metal articles, comprising casting the metal to form an ingot having a body portion and flanges thereon, separating the flanges from

the body portion and forming the article from the flanges.

2. The method of making non-porous metal articles, comprising casting a solid ingot having a body portion of relatively porous metal and flanges of relatively non-porous metal, separating the flanges from the body portion and forming the article from the flanges.

10 3. The method of making non-porous steel pistons for pneumatic hammers and drills, comprising casting a steel ingot having a body portion and flanges thereon, separating the flanges from the body portion, and forming the flanges into pistons.

15 4. The method of making non-porous metal articles, comprising casting the metal to form an ingot having a body portion and flanges thereon, longitudinally separating the flanges from the body portion, and forming the article from the flanges.

20 5. The method of making non-porous metal articles, comprising casting the metal to form an ingot having a body portion and flanges extending therefrom, the flanges and body portion being connected throughout the major portion thereof, longitudinally separating the flanges from the body portion, and forming the article from the flanges.

25 6. The method of making non-porous metal articles, comprising casting the metal to form an ingot having a body portion and flanges extending therefrom, the flanges and body portion being connected throughout substantially their entire lengths, longitudinally separating the flanges from the body portion, and forming the article from the flanges.

30 In testimony whereof I have hereunto set  
40 my hand.

L. GERALD FIRTH.

the body portion and forming the article from the flanges.

2. The method of making non-porous metal articles, comprising casting a solid ingot having a body portion of relatively porous metal and flanges of relatively non-porous metal, separating the flanges from the body portion and forming the article from the flanges.
- 5 3. The method of making non-porous steel pistons for pneumatic hammers and drills, comprising casting a steel ingot having a body portion and flanges thereon, separating the flanges from the body portion, and forming the flanges into pistons.
- 10 4. The method of making non-porous metal articles, comprising casting the metal to form an ingot having a body portion and flanges thereon, longitudinally separating the flanges from the body portion, and forming the article from the flanges.
- 15 5. The method of making non-porous metal articles, comprising casting the metal to form an ingot having a body portion and flanges extending therefrom, the flanges and body portion being connected throughout the major portion thereof, longitudinally separating the flanges from the body portion, and forming the article from the flanges.
- 20 6. The method of making non-porous metal articles, comprising casting the metal to form an ingot having a body portion and flanges extending therefrom, the flanges and body portion being connected throughout substantially their entire lengths, longitudinally separating the flanges from the body portion, and forming the article from the flanges.

30 In testimony whereof I have hereunto set my hand.

L. GERALD FIRTH.

**CERTIFICATE OF CORRECTION.**

Patent No. 1,792,581.

Granted February 17, 1931, to

It is hereby certified that the christian name of the patentee in the above numbered patent was erroneously written and printed as "Louis" whereas said name should have been written and printed Lewis; and that the said Letters Patent should be read with this correction therein that the same may conform to the record of the case in the Patent Office.

Signed and sealed this 17th day of March, A. D. 1931.

(Seal)

**M. J. Moore,**  
Acting Commissioner of Patents.

**CERTIFICATE OF CORRECTION.**

**Patent No. 1,792,581.**

**Granted February 17, 1931, to**

**It is hereby certified that the christian name of the patentee in the above numbered patent was erroneously written and printed as "Louis" whereas said name should have been written and printed Lewis; and that the said Letters Patent should be read with this correction therein that the same may conform to the record of the case in the Patent Office.**

**Signed and sealed this 17th day of March, A. D. 1931.**

**(Seal)**

**M. J. Moore,  
Acting Commissioner of Patents.**